



US005747205A

**United States Patent** [19]**Hu et al.**[11] **Patent Number:** **5,747,205**[45] **Date of Patent:** **May 5, 1998**[54] **PHOTOCONDUCTIVE IMAGING MEMBERS**[75] Inventors: **Nan-Xing Hu**, Oakville; **Ping Liu**; **Beng S. Ong**, both of Mississauga, all of Canada[73] Assignee: **Xerox Corporation**, Stamford, Conn.[21] Appl. No.: **807,487**[22] Filed: **Feb. 27, 1997**[51] Int. Cl.<sup>6</sup> ..... **G03G 5/047**[52] U.S. Cl. ..... **430/59**; 430/73; 430/79

[58] Field of Search ..... 430/59, 79, 73

[56] **References Cited**

## U.S. PATENT DOCUMENTS

|           |         |                 |       |         |
|-----------|---------|-----------------|-------|---------|
| 4,356,429 | 10/1982 | Tang            | ..... | 313/503 |
| 4,539,507 | 9/1985  | VanSlyke et al. | ..... | 313/504 |
| 4,769,292 | 9/1988  | Tang et al.     | ..... | 428/690 |
| 4,950,950 | 8/1990  | Perry et al.    | ..... | 313/504 |
| 5,150,006 | 9/1992  | VanSlyke et al. | ..... | 313/504 |
| 5,495,049 | 2/1996  | Nukada et al.   | ..... | 564/433 |
| 5,654,482 | 8/1997  | Goodbrand       | ..... | 564/405 |

*Primary Examiner*—John Goodrow*Attorney, Agent, or Firm*—E. O. Palazzo[57] **ABSTRACT**

A photoconductive imaging member comprised of a starburst aromatic amine compound of the formula



wherein N is nitrogen; A<sup>1</sup> to A<sup>3</sup> each individually represent biaryl; R<sub>a</sub>, R<sub>b</sub>, and R<sub>c</sub> independently represent one of the groups of the following formulas



wherein N is nitrogen; each Ar<sup>1</sup> and Ar<sup>2</sup> are aryl; R<sub>1</sub> to R<sub>8</sub> are substituents independently selected from the group consisting of hydrogen, halogen, hydrocarbon, and alkoxy; and X represents oxygen, sulfur, or an alkylene.

**8 Claims, No Drawings**

## PHOTOCONDUCTIVE IMAGING MEMBERS

## PENDING APPLICATIONS

Illustrated in copending application U.S. Ser. No. 08/807510 are EL devices with starburst amines, the disclosure of this application being totally incorporated herein by reference.

## BACKGROUND OF THE INVENTION

This invention is generally directed to photoconductive imaging members with starburst amines and processes thereof, and to electroluminescent (EL) devices. More specifically, this invention is directed to organic EL devices with enhanced thermal and operational stability, and thus improved durability, and which devices utilize novel hole transport compositions comprised of starburst aromatic amines. In embodiments, the present invention relates to processes for the preparation of starburst aromatic amines, and which amines may be selected for photoconductive imaging members, especially layered imaging members, and wherein the starburst amines function primarily as charge transport components, or molecules, reference the photoconductive imaging members illustrated in U.S. Pat. No. 4,265,990, the disclosure of which is totally incorporated herein by reference.

## PRIOR ART

Layered photoconductive imaging members with certain charge transport aryl amines are illustrated in a number of patents, such as U.S. Pat. No. 4,265,990, the disclosure of which is totally incorporated herein by reference.

With respect to prior art organic EL devices, they can be comprised of a laminate of an organic luminescent material and electrodes of opposite polarity, which devices include a single crystal material, such as single crystal anthracene, as the luminescent substance as described, for example, in U.S. Pat. No. 3,530,325. However, these devices require excitation voltages on the order of 100 volts or greater. Subsequent modifications of the device structure through incorporation of additional layers, such as charge injecting and charge transport layers, have led to performance improvement. More recently, organic EL devices comprised of multi-layered thin films of organic materials provide advantages including low operating voltages and high luminance of greater than a few hundred cd/m<sup>2</sup>. Illustrative examples of these type of EL devices have been disclosed in publications by Tang et al. in *J. Appl. Phys.* vol. 65, pp. 3610 to 3616 (1989) and Saito et al. in *Mol. Cryst. Liq. Cryst.* vol. 253, pp. 125 to 132 (1994), the disclosures of which are totally incorporated herein by reference. Moreover, U.S. Pat. No. 4,950,950 illustrates a multilayer EL device with silane hole transporting agents. U.S. Pat. No. 4,356,429 illustrates organic EL cells with a hole injecting porphyrinic layer.

An EL device with an organic dual layer structure comprises one layer adjacent to the anode supporting hole injection and transport, and another layer adjacent to the cathode supporting electron injection and transport. The recombination of charge carriers and subsequent emission of light occurs in one of the layers near the interface between the two layers. Optionally, a fluorescent material capable of emitting light in response to recombination of holes and electrons can be added to one of the layers. In another configuration, an EL device can comprise three separate layers, a hole transport layer, an emission layer, and an electron transport layer, which are laminated in sequence and are sandwiched as a whole between an anode and a cathode.

Although recent performance improvements in organic EL devices have suggested a potential for widespread use, most practical applications require limited operation voltage or light output variance over an extended period of time. 5 Many current organic EL devices possess limited operational lifetime, particularly at a high temperature of, for example, above 40° C. (Centigrade). One aspect which significantly affects the performance of organic EL devices is the thermal and morphological stability of the organic 10 layers comprising the devices. These layers are amorphous thin films formed by vacuum deposition technique. The transition of an organic thin film from an amorphous state to a crystalline state can result in a physical or morphological change in the thin film. The integrity of organic EL devices 15 with multi-layer structures is sensitive to this morphological change primarily because the charge carriers transport characteristics are substantially affected by the microscopic structures of the organic layers. Since the transition is generally dependent on temperature, a transition temperature 20 from an amorphous state to a crystalline state is known as a glass transition temperature T<sub>g</sub>. Thus, to improve the thermal and operation stability of organic EL devices, it is important that the organic materials comprising the layers in the devices should possess high glass transition temperatures. 25

## SUMMARY OF THE INVENTION

Examples of objects include:

It is an object of the present invention to provide photoconductive imaging members, starburst amines, and processes thereof illustrated herein.

Another object of the present invention is the provision of certain starburst aromatic amine compounds for photoconductive members, which compounds have a high glass transition temperature of, for example, above 100° C., and a process for the preparation of the starburst aromatic amines.

In embodiments, the present invention also relates to EL devices that are comprised in the following order of an anode, a hole injecting and transporting zone or layer, an electron injecting and transporting zone or layer, and a cathode, and wherein the hole injecting and transporting zone is comprised of a starburst aromatic amine represented by the following Formula



wherein N is nitrogen; A<sup>1</sup> to A<sup>3</sup> individually represent a biaryl with, for example, from 12 to about 60 carbon atoms, 55 such as a biphenyl group or a bitolyl group; R<sub>a</sub>, R<sub>b</sub>, and R<sub>c</sub>, represent independently one of the following functional groups of the formulas indicated and wherein N is nitrogen; Ar<sup>1</sup> and Ar<sup>2</sup> are aryl groups with, for example, from 6 to about 24 carbon atoms, such as a phenyl group, a tolyl group, a halo, such as chlorophenyl group, an alkoxy, such as a methoxyphenyl group, a biphenyl group, or a naphthyl group and the like; R<sub>1</sub> to R<sub>8</sub> are substituents independently selected from the group consisting of hydrogen, halogen, or hydrocarbon groups, for example from 1 to 10 carbon atoms, 60 and alkoxy groups containing, for example, from 1 to 6 carbon atoms; and X represents an oxygen atom, a sulfur atom, or an alkylene like a methylene group.



and bidentate tertiary amines. The reaction is generally accomplished in an inert solvent, such as toluene, xylene, mesitylene, dodecane, and the like, at a temperature ranging, for example, from about 100° C. to about 190° C., and preferably from about 120° C. to about 160° C., in the presence of a ligated copper catalyst, such as 1,10-phenanthrolato copper (1) (monovalent) chloride, dipyridino copper (1) chloride, 1,10-phenanthrolato copper (1) bromide, dipyridino copper (1) bromide, 1,10-phenanthrolato copper (1) chloride, 1,10-phenanthrolato copper (1) bromide, or dipyridino copper (1) bromide. The catalyst selected is of importance and in embodiments is comprised of a copper containing organic ligand, and wherein the ligand is selected from the group consisting of monodentate tertiary amines and bidentate tertiary amines as indicated herein, and more specifically, copper catalysts or compounds, such as (1,10-phenanthrolato) Cu(X) and bis (pyridinato)Cu(X), wherein X is a halide, such as chloride. Ligation of the copper salt dramatically increases catalyst efficiency permitting very rapid reactions to occur, generally over about several hours, at lower temperatures.

The important catalyst selected for the processes of the present invention is as illustrated herein, and in embodiments is comprised of ligated copper salts, including the halide salts, such as chloride, bromide, iodide, and fluoride, especially copper (1), and wherein the ligands are monodentate tertiary amines, or bidentate tertiary amines, such as 1,10-phenanthroline or pyridine. The amount of catalyst selected can vary, and generally, the catalyst is employed in effective amounts, such as from about 1 to about 20 mole percent of the reactants, and preferably from about 5 to about 12 mole percent of the limiting reactant. Examples of postulated formula structures for the copper catalysts include



wherein X denotes a halide such as chloride or bromide.

The catalysts can be prepared as illustrated in the relevant copending applications recited herein, and more specifically, by the reaction of a copper salt like cuprous chloride with the appropriate ligand like 1,10-phenanthroline, and which reaction is accomplished with heating, for example, from about 70° C. to about 125° C. The reaction mixture is cooled and the product catalyst may, it is believed, be isolated by, for example, filtration. Preferably, the catalyst is prepared in situ.

Specific examples of starburst aromatic amines include (1) tris[4'-(phenyl-m-tolylamino)-1,1'-biphenyl-4-yl]amine, (2) N,N-bis(4'-di-m-tolylamino-1,1'-biphenyl-4-yl)-N',N'-diphenylbenzidine, (3) tris[4'-(m-methoxydiphenylamino)-1,1'-biphenyl-4-yl]amine, (4) tris[4'-(diphenylamino) 1,1'-biphenyl-4-yl]amine, (5) tris[4'-(carbazol-9-yl)-1,1'-biphenyl-4-yl]amine, (6) tris[4'-(1-naphthylphenylamino)-1,1'-biphenyl-4-yl]amine, (7) N,N-bis[4'-(phenyl-m-tolylamino)-1,1'-biphenyl-4-yl]-N'-phenyl-N'-m-tolyl-3,3'-dimethylbenzidine, (8) N,N-bis(4'-diphenylamino-1,1'-biphenyl-4-yl)-N'-phenyl-N'-m-tolyl-3,3'- (9) N,N-bis(diphenylamino-1,1'-biphenyl-4-yl)-N'-phenyl-N'-m-tolylbenzidine, (10) N,N-bis[4'-(di-m-tolylamino)-1,1'-biphenyl-4-yl]-N'-phenyl-N'-p-tolylbenzidine, (11) tris[4'-(8H-10H-acridin-10-yl)-1,1'-biphenyl-4-yl]amine, (12) tris[4'-(9,9-dimethyl-9H-10H-acridin-10-yl)-1,1'-biphenyl-4-yl]amine, (13) tris[4'-phenoxyazin-10-yl-1,1'-biphenyl-4-yl]amine, (14) tris[4'-phenoxyazin-10-yl-1,1'-biphenyl-4-yl]amine, (15) N,N-bis[4'-(phenyl-m-tolylamino)-1,1'-biphenyl-4-yl]-4'-(carbazol-9-yl)-1,1'-biphenyl-4-amine, (16) N,N-bis[4'-(carbazol-9-yl)-1,1'-biphenyl-4-yl]-N'-phenyl-N'-m-tolylbenzidine, (17) N,N-bis[4'-(1naphthylphenylamino)-1,1'-biphenyl-4-yl]-4'-(carbazol-9-yl)-1,1'-biphenyl-4-amine, (18) N,N-bis[4'-(9H-10H-acridin-10-yl)-1,1'-biphenyl-4-yl]-4'-(9H-10H-acridin-10-yl)-1,1'-biphenyl-4-yl]-4'-(9H-10H-acridin-10-yl)-1,1'-biphenyl-4-amine, and the like.

5,747,205

7



8

(1)



(2)

**9****10**

-continued



(3)



(4)

-continued



(5)



(6)

-continued



(7)



(8)

**15****16**

-continued



(9)



(10)

5,747,205

17

18

-continued



(11)



(12)

-continued



(13)



(14)

-continued



(15)



(16)



(17)



(18)



With respect to EL devices the hole injecting and hole transporting zone can be entirely formed of a single layer comprised of an aforementioned starburst aromatic amine. Further, it can be advantageous for the hole injecting and transporting zone to be comprised of a starburst aromatic amine in combination with a porphyrinic compound or a tetraarylamine compound. When a starburst aromatic amine in effective amounts, such as from about 75 to about 95 weight percent, is utilized in combination with a porphyrinic compound, the porphyrinic can be a compound positioned as a layer interposed between the anode and the starburst aromatic amine layer. Examples of porphyrinic compounds are porphyrine; 1,10,15,20-tetraphenyl-21H,23H-porphyrin

55

copper (II); copper phthalocyanine, copper tetramethyl phthalocyanine; zinc phthalocyanine; titanium phthalocyanine oxide; magnesium phthalocyanine; and the like.

When the starburst aromatic amine compound of an EL device is selected in combination with a triarylamine, tetraarylamine, and the like in forming the hole injecting and transporting zone, the amine is positioned as a layer, for example at a thickness of from about 200 Angstroms, 60 interposed between the starburst aromatic amine layer and the electron injecting and transporting zone. Illustrative examples of aromatic tertiary amines are as illustrated in the relevant copending applications recited herein, and include the following



wherein Ar<sup>1</sup> to Ar<sup>4</sup> are aryl groups with, for example, 6 to about 30 carbon atoms, and, for example, independently selected from phenyl, tolyl, xylyl, naphthyl, 4-biphenyl, and the like; P is an arylene like a phenylene group; and n is an integer of from 1 to 4. Specific examples include N,N'-diphenyl-N,N'-bis (3-methylphenyl)-1,1'-biphenyl-4,4'-diamine, N,N'-diphenyl-N,N'-bis (4-methylphenyl)-1,1'-biphenyl-4,4'-diamine, N,N',N',N'-tetra-p-tolyl-1,1'-biphenyl-4,4'-diamine, N,N'-di-1-naphthyl-N,N'-diphenyl-1,1'-biphenyl-4,4'-diamine, N,N'-di-2-naphthyl-N,N'-diphenyl-1,1'-biphenyl-4,4'-diamine, N,N'-di-1-naphthyl-N,N'-bis(3-methylphenyl)-1,1'-biphenyl-4,4'-diamine, N,N'-di-1-naphthyl-1-N,N'-bis (4-methylphenyl)-1,1'-biphenyl-4,4'-diamine, N,N'-di-4-biphenyl-1-N,N'-bis (4-methylphenyl)-1,1'-biphenyl-4,4'-diamine, N,N'-di-4-biphenyl-1-N,N'-bis (4-methylphenyl)-1,1'-biphenyl-4,4'-diamine, and the like.

The electron injecting and transporting zone in the EL devices of the present invention can be comprised of any conventional electron injecting and transporting compound or compounds. Examples of useful electron transport compounds include fused ring luminescent materials such as anthracene, phenanthrene, pyrene, perylene, and the like as illustrated by U.S. Pat. No. 3,172,862; butadienes such as 1,4-diphenylbutadiene and tetraphenylbutadiene, and stilbenes, and the like as illustrated in U.S. Pat. Nos. 4,356,429 and 5,516,577; optical brightness such as those disclosed by U.S. Pat. No. 4,539,507.

Particularly preferred electron transport materials are metal chelates of 8-hydroxyquinoline disclosed in U.S. Pat. No. 4,539,507; 5,151,629, and 5,150,006. Illustrative examples of the metal chelated compounds include tris(8-hydroxyquinolinate)aluminum (AIQ3), tris(8-hydroxyquinolinate)gallium, bis(8-hydroxyquinolinate)magnesium, bis(8-hydroxyquinolinate)zinc, tris(5-methyl-8-hydroxyquinolinate)aluminum, tris(7-propyl-8-quinololato)aluminum, bis[benzo{f}-8-quinolinate]zinc, bis(10-hydroxybenzo[h]quinolinate)beryllium, bis(2-methylquinololato)aluminum (III)-μ-oxo-bis(2-methyl-8-quinololato)aluminum(III), bis(2-methyl-8-quinololato)(phenolato)aluminum, bis(2-methyl-8-quinololato)(para-phenylphenolato)aluminum, bis(2-methyl-8-quinololato)(2-naphthalolato)aluminum and the like.

The disclosures of each of the above patents are totally incorporated herein by reference.

Another class of preferred electron injecting and transporting compounds is metal thioxinoid compounds, disclosed in copending application U.S. Ser. No. 609,259. Illustrative examples of metal thioxinoid compounds include bis(8-quinolinethiolato), bis(8-quinolinethiolato) cadmium, tris(8-quinolinethiolato)gallium, tris(8-quinolinethiolato) indium, bis(5-methylquinolinethiolato) zinc, tris(5-methylquinolinethiolato) gallium, tris(5-methylquinolinethiolato)indium, bis(5-methylquinolinethiolato) cadmium, bis(3-methylquinolinethiolato)cadmium, bis(5-methylquinolinethiolato)zinc, bis[benzo{f}-8-quinolinethiolato]zinc, bis[3-methylbenzo{f}-8-quinolinethiolato]zinc, bis[3,7-dimethylbenzo{f}-8-quinolinethiolato]zinc, and the like.

In embodiments of the present invention, the total thickness of the organic luminescent medium, which includes the

hole injecting and transporting zone and the electron injecting and transporting zone, is preferably, for example, less than about 1 micron, for example from about 0.05 to about 1 micron, to maintain a current density compatible with an efficient light emission under a relatively low voltage applied across the electrodes. Suitable thickness of the hole injecting and transporting zone can range from about 50 to about 2,000 Å, and preferably from about 400 to 1,000 Å. Similarly, the thickness of the electron injecting and transporting zone can range from about 50 to about 2,000 Å, and preferably from about 400 to 1,000 Å.

The cathode can be constructed of any metal, including high or low work function metals. The cathode which can be derived from a combination of a low work function metal, for example less than about 4 eV, for example from about 2 to about 4, and at least one second metal can provide additional advantages such as improved device performance and stability. Suitable proportions of the low work function metal to the second metal may range from less than about 0.1 percent to about 99.9 percent by weight, and in embodiments are from about 1 to about 90 weight percent. Illustrative examples of low work function metals include alkaline metals, Group 2A or alkaline earth metals, and Group III metals including rare earth metals and the actinide group metals. Lithium, magnesium and calcium are particularly preferred.

The thickness of cathode ranges from, for example, about 10 to about 5,000 Å, and more specifically, from about 50 to about 250 Angstroms. The Mg:Ag cathodes of U.S. Pat. No. 4,885,211 constitute one preferred cathode construction. Another preferred cathode construction is described in U.S. Pat. No. 5,429,884, wherein the cathodes are formed from lithium alloys with other high work function metals such as aluminum and indium. The disclosures of each of the patents are totally incorporated herein by reference.

Both the anode and cathode of the organic EL devices of the present invention can be of any convenient form. A thin, for example about 200 Angstroms, conductive anode layer can be coated onto a light transmissive substrate, for example, a transparent or substantially transparent glass plate or plastic film. The EL device can include a light transmissive anode formed from tin oxide or indium tin oxide coated on a glass plate. Also, very thin, for example less than 200 Å, such as from about 50 to about 175 Angstroms, light-transparent metallic anodes can be selected, such as gold, palladium, and the like. In addition, transparent or semitransparent thin, for example 200 Angstroms, conjugated polymers, such as polyaniline, polypyrrole, and the like, can be selected. Any light transmissive polymeric film, for example from about 50 to about 200 Angstroms in thickness, can be selected as the substrate. Further, suitable forms of the anode and cathode are illustrated by U.S. Pat. No. 4,885,211, the disclosure of which is totally incorporated herein by reference.

The photoconductive imaging member can be comprised of a supporting substrate, such as MYLAR®, polymers, metals like aluminum, and thereover a photogenerating layer containing known photogenerating pigments, such as phthalocyanines, selenium, hydroxygallium phthalocyanines, titanyl phthalocyanines, perylenes, and the like, and which pigments can be dispersed in resin binders. In contact with the photogenerating layer and situated thereover or thereunder is a charge transport layer comprised of the starburst amines illustrated herein, and which amines may be dispersed in resin binders. The resin binders, thickness of each of the layers, and amounts of components selected for each layer, other layers present, and the like are illustrated in a number of issued United States patents, such

as U.S. Pat. Nos. 4,265,990; 4,585,884; 4,584,253; 4,563,408; 4,587,189; 4,555,463; 5,153,313; 5,614,493, and 5,189,155; and in U.S. Ser. No. 700,326, the disclosures of each of these patents and patent application being totally incorporated herein by reference. For example, the supporting substrate of MYLAR® is coated with a photogenerating layer containing a photogenerating pigment, 100 weight percent, or 95 weight percent, and 5 weight percent resin binder, and coated thereover a charge transport layer containing the starburst amines illustrated herein.

The following Examples are provided.

#### EXAMPLE I

##### Synthesis of Tris[4'-(phenyl-m-tolylamino)-1,1'-biphenyl-4-yl]amine-Compound (1)

A 250 milliliter 3-necked round bottom flask equipped with a mechanical stirrer, reflux condenser, and argon inlet was purged with argon and then charged with N-phenyl-N-m-tolyl benzidine (8.0 grams, 0.023 mol), 4'-iodo-N-phenyl-N-m-tolyl-4-aminobiphenyl (17.5 grams, 0.038 mol), xylene (15 milliliters), 1,10-phenanthroline (0.34 gram, 1.9 mmol), cuprous chloride (0.188 gram, 1.9 mmol), and potassium hydroxide flakes (17.06 grams, 0.3 mol). Under an argon atmosphere, the reaction mixture was heated to reflux with an oil bath and allowed to proceed at that temperature until chromatographic analysis indicated that the reaction was complete after approximately 6 hours. The oil bath was removed and 100 milliliters of toluene and 25 milliliters of water were then added with efficient stirring. The resulting two phase mixture was transferred into a separatory funnel and the layers separated. The organic phase was washed with water and treated under argon with 25 grams of alumina. After the alumina was filtered off, the organic phase was evaporated to remove most of the toluene. The above product, Compound (1), was obtained by recrystallization of the residue from cyclohexane. Yield: 12.3 grams; m.p. 234.28° C.; Tg 134° C.

#### EXAMPLE II

##### Synthesis of N,N-bis(4'-di-m-tolylamino)-1,1'-biphenyl-4-yl)-N,N'-diphenylbenzidine-Compound (2)

A 250 milliliter 3-necked round bottom flask equipped with a mechanical stirrer, reflux condenser, and argon inlet was purged with argon and then charged with N,N-diphenylbenzidine (6.056 grams, 0.009 mol), 4'-iodo-N-phenyl-N-m-tolyl-4-aminobiphenyl (6.734 grams, 0.015 mol), xylene (10 milliliters), 1,10-phenanthroline (0.135 gram, 0.75 mmol), cuprous chloride (0.074 gram, 0.75 mmol), and potassium hydroxide flakes (6.73 grams, 0.12 mol). Under an argon atmosphere, the reaction mixture was heated to reflux with an oil bath and allowed to proceed at that temperature until chromatographic analysis indicated that the reaction was complete after approximately 6 hours. The oil bath was removed and 100 milliliters of toluene and 10 milliliters of water were then added with efficient stirring. The resulting two phase mixture was transferred into a separatory funnel and the layers separated. The organic phase was washed with water and treated under argon with 20 grams of alumina. After the alumina was filtered off, the organic phase was evaporated to remove most of the toluene. The above product compound was obtained by recrystallization of the residue from cyclohexane. Yield: 8.75 grams; m.p. 254.5° C.; Tg 128° C.

#### EXAMPLE III

##### Synthesis of Tris[4'-(m-methoxydiphenylamino)-1,1'-biphenyl-4-yl]amine-Compound (3)

A 250 milliliter 3-necked round bottom flask equipped with a mechanical stirrer, reflux condenser, and argon inlet

was purged with argon and then charged with N-methoxyphenyl-N-phenylbenzidine (6.2 grams, 0.017 mol), 4'-iodo-N-m-methoxyphenyl-N-phenyl-4-aminobiphenyl (13.49 grams, 0.028 mol), xylene (15 milliliters), 1,10-phenanthroline (0.252 gram, 1.4 mmol), cuprous chloride (0.139 gram, 1.4 mmol), and potassium hydroxide flakes (12.57 grams, 0.224 mol). Under an argon atmosphere, the reaction mixture was heated to reflux with an oil bath and allowed to proceed at that temperature until chromatographic analysis indicated that the reaction was complete after approximately 8 hours. The oil bath was removed and 100 milliliters of toluene and 25 milliliters of water were then added with efficient stirring. The resulting two phase mixture was transferred into a separatory funnel and the layers separated. The organic phase was washed with water and treated under argon with 20 grams of alumina. After the alumina was filtered off, the organic phase was evaporated to remove most of the toluene. The crude product was further chromatographed on silica gel using a 10:1 hexane-toluene as an eluent to provide pure tris[4-(3-methoxydiphenylamino)-1,1'-biphenyl]amine as amorphous powder. Yield: 10.1 grams.

#### EXAMPLE IV

##### Synthesis of Tris[4'-(diphenylamino)-1,1'-biphenyl-4-yl]amine -Compound(4)

A 250 milliliter 3-necked round bottom flask equipped with a mechanical stirrer, reflux condenser, and argon inlet was purged with argon and then charged with N,N-diphenylbenzidine (4.95 grams, 0.0147 mol), 4'-iodo-N,N-diphenyl-4-aminobiphenyl (11.0 grams, 0.0246 mol), xylene (15 milliliters), 1,10-phenanthroline (0.22 gram, 1.22 mmol), cuprous chloride (0.122 gram, 1.22 mmol), and potassium hydroxide flakes (11.04 grams, 0.197 mol). Under an argon atmosphere, the reaction mixture was heated to reflux with an oil bath and allowed to proceed at that temperature until chromatographic analysis indicated that the reaction was complete after approximately 6 hours. The oil bath was removed and 100 milliliters of toluene and 20 milliliters of water were then added with efficient stirring. The resulting two phase mixture was transferred into a separatory funnel and the layers separated. The organic phase was washed with water and treated under argon with 25 grams of alumina. After the alumina was filtered off, the organic phase was evaporated to remove the toluene. The above product compound was obtained by recrystallization of the residue from cyclohexane. Yield: 6.9 grams. m.p. 283.97° C., Tg 141° C.

#### EXAMPLE V

##### Synthesis of Tris[4'-(carbazol-9-yl)-1,1'-biphenyl-4-yl]amine-Compound (5)

A 250 milliliter 3-necked round bottom flask equipped with a mechanical stirrer, reflux condenser, and argon inlet was purged with argon and then charged with 4'-(9-carbazolyl)-4-aminobiphenyl (5.1 grams, 0.0153 mol), 4-(9-carbazolyl)-4'-iodo-1,1'-biphenyl (11.394 grams, 0.0255 mol), 1,3,5-trimethylbenzene (15 milliliters), 1,10-phenanthroline (0.23 gram, 1.28 mmol), cuprous chloride (0.126 gram, 1.28 mmol), and potassium hydroxide flakes (11.45 grams, 0.204 mol). Under an argon atmosphere, the reaction mixture was heated to reflux with an oil bath and allowed to proceed at that temperature until chromatographic analysis indicated that the reaction was complete after approximately 12 hours. The oil bath was removed and

150 milliliters of toluene and 15 milliliters of water were then added with efficient stirring. The resulting two phase mixture was transferred into a separatory funnel and the layers separated. The organic phase was washed with water and treated under argon with 20 grams of alumina. After the alumina was filtered off, the organic phase was evaporated to remove most of the toluene. The residue was chromatographed on silica gel using 10:1 cyclohexane-dichloromethane as an eluent to provide 2.1 grams of the product compound. m.p. 283.13° C.

With respect to EL Devices:

#### EXAMPLE VI

An organic EL was prepared as illustrated in the relevant copending applications recited herein, and for example, in the following manner:

1. An indium tin oxide, 500 Angstroms, (ITO) coated glass, (1 millimeter) was cleaned with a commercial detergent, rinsed with deionized water and dried in a vacuum oven at 600° C. for 1 hour. Immediately before use, the glass was treated with UV ozone for 0.5 hour.

2. The ITO substrate was placed in a vacuum deposition chamber. The deposition rate and layer thickness were controlled by an Inficon Model IC/5 controller. Under a pressure of slightly less than about  $5 \times 10^{-6}$  Torr a starburst aromatic amine, such as those of Examples I to IV, was evaporated from an electrically heated tantalum boat to deposit an 80 nanometer hole transport layer on the ITO glass layer 1. The deposition rate of the amine compound was controlled at 0.6 nanometer/second.

3. Onto the transport layer of 2 was deposited tris(8-hydroxyquinolinolate) aluminum at an evaporation rate of 0.6 nanometer/second to form an 80 nanometer electron injecting and transporting layer.

4. A 100 nanometer magnesium silver alloy was deposited at a total deposition rate of 0.5 nanometer/second onto the electron injecting and electron transporting layer of 3 by simultaneous evaporation from two independently controlled tantalum boats containing Mg and Ag, respectively. The typical composition was 9:1 in atomic ratio of Mg to Ag. Finally, a 200 nanometer silver layer was overcoated on the Mg:Ag cathode for the primary purpose of protecting the reactive Mg from ambient moisture.

The devices as prepared above were retained in a dry box which was continuously purged with nitrogen gas. The performance of the devices was assessed by measuring its current-voltage characteristics and light output under a direct current measurement. The current-voltage characteristics were determined with a Keithley Model 238 High Current Source Measure Unit. The ITO electrode was always connected to the positive terminal of the current source. At the same time, the light output from the device was monitored by a silicon photodiode.

The performance characteristics of the devices were evaluated under a constant current density of 33 mA/cm<sup>2</sup>. The operation life was measured by a sustained operation time in which the light intensity reduced to a half level of the initial intensity. The initial light intensity and operation life of the devices utilizing starburst amine compounds (1) to (5) are summarized in the following table.

| Compound No. | $L_0$ (cd/m <sup>2</sup> ) | Operation life (hours) |
|--------------|----------------------------|------------------------|
| 1            | 750                        | 230                    |
| 2            | 730                        | 250                    |
| 3            | 810                        | 150                    |
| 4            | 720                        | 245                    |
| 5            | 510                        | 260                    |

These results demonstrate that a sustained high level of light output can be achieved in the organic EL devices comprising a starburst aromatic amine hole transport component. Furthermore, an organic EL device utilizing the starburst aromatic amine compound (2) as the hole transporting layer displayed no change in its current-light intensity characteristics even after it was subjected to a temperature of 60° C. for 72 hours.

Photoconductive layered devices can be prepared as illustrated herein, and more specifically as illustrated in the relevant United States patents recited herein, and in U.S. Ser. No. 700,326, the disclosures each of which are totally incorporated herein by reference, and wherein the starburst amine functions as the charge transport component.

Other modifications of the present invention will occur to those of ordinary skill in the art subsequent to a review of the present application. These modifications, and equivalents thereof, are intended to be included within the scope of the invention.

What is claimed is:

1. A photoconductive imaging member comprised of a starburst aromatic amine compound of the formula



wherein N is nitrogen; A<sup>1</sup> to A<sup>3</sup> each individually represent aryl; R<sub>a</sub>, R<sub>b</sub>, and R<sub>c</sub> independently represent one of the groups of the following formulas





wherein N is nitrogen; each Ar<sup>1</sup> and Ar<sup>2</sup> are aryl; R<sub>1</sub> to R<sub>8</sub> are substituents independently selected from the group consisting of hydrogen, halogen, hydrocarbon, and alkoxy; and X represents oxygen, sulfur, or an alkylene.

2. A member in accordance with claim 1 wherein the aromatic amine is present as a layer on the photogenerating layer, and wherein the photogenerating layer is present on a supporting substrate, or wherein the aromatic amine is present on said substrate, and wherein said hydrocarbon contain from 1 to about 10 carbon atoms, and said alkoxy contains from 1 to about 6 carbon atoms.

3. A member in accordance with claim 1 wherein the aromatic amine is selected from the group consisting of tris[4'-(phenyl-m-tolylamino)-1,1'-biphenyl-4-yl]amine; N,N-bis(4'-di-m-tolylamino-1,1'-biphenyl-4-yl)-N',N'-diphenylbenzidine; tris[4'-(m-methoxydiphenylamino)-1,1'-biphenyl-4-yl]amine; tris[4'-(diphenylamino)-1,1'-biphenyl-4-yl]amine; tris[4'-(carbazol-9-yl)-1,1'-biphenyl-4-yl]amine; tris[4'-(1-naphthylphenylamino)-1,1'-biphenyl-4-yl]amine; N,N-bis[4'-(phenyl-m-tolylamino)-1,1'-biphenyl-4-yl]-N'-phenyl-N'-m-tolyl-3,3'-dimethylbenzidine; N,N-bis(4'-diphenylamino-1,1'-biphenyl-4-yl)-N'-phenyl-N'-m-tolyl-3,3'-dimethylbenzidine; N,N-bis(diphenylamino-1,1'-biphenyl-4-yl)-N'-phenyl-N'-m-tolylbenzidine; N,N-bis[4'-(di-m-tolylamino)-1,1'-biphenyl-4-yl]-N'-phenyl-N'-p-tolylbenzidine; tris[4'-(8H-10H-acridin-10-yl)-1,1'-biphenyl-4-yl]amine; tris[4'-(9,9-dimethyl-9H-10H-acridin-10-yl)-1,1'-biphenyl-4-yl]amine; tris[4'-phenoxy-10-yl-1,1'-biphenyl-4-yl]amine; tris[4'-phenoxy-10-yl-1,1'-biphenyl-4-yl]amine; N,N-bis[4'-(phenyl-m-tolylamino)-1,1'-biphenyl-4-yl]-N'-phenyl-N'-m-tolylbenzidine; N,N-bis[4'-(1-naphthylphenylamino)-1,1'-biphenyl-4-yl]-N'-carbazol-9-yl)-1,1'-biphenyl-4-amine; and N,N-bis[4'-(9H-10H-acridin-10-yl)-1,1'-biphenyl-4-yl]-N'-carbazol-9-yl)-1,1'-biphenyl-4-amine.

**32**

yl)-1,1'-biphenyl-4-amine; N,N-bis[4'-(carbazol-9-yl)-1,1'-biphenyl-4-yl]-N'-phenyl-N'-m-tolylbenzidine; N,N-bis[4'-(1-naphthylphenylamino)-1,1'-biphenyl-4-yl]-N'-carbazol-9-yl)-1,1'-biphenyl-4-amine; and N,N-bis[4'-(9H-10H-acridin-10-yl)-1,1'-biphenyl-4-yl]-N'-carbazol-9-yl)-1,1'-biphenyl-4-amine.

4. A member in accordance with claim 2 wherein the photogenerating layer contains photogenerating pigments of metal phthalocyanines or metal free phthalocyanines.

10 5. A member in accordance with claim 2 wherein the photogenerating layer contains photogenerating pigments of perylenes, titanyl phthalocyanines, hydroxygallium phthalocyanines, or vanadyl phthalocyanines.

15 6. A member in accordance with claim 2 wherein said photogenerating layer is comprised of photogenerating pigments dispersed in a resin binder.

7. A member in accordance with claim 2 wherein said amine is dispersed in an inactive resin binder.

20 8. A member in accordance with claim 2 wherein said amine is selected from the group consisting of tris[4'-(phenyl-m-tolylamino)-1,1'-biphenyl-4-yl]amine; N,N-bis(4'-di-m-tolylamino-1,1'-biphenyl-4-yl)-N',N'-diphenylbenzidine; tris[4'-(m-methoxydiphenylamino)-1,1'-biphenyl-4-yl]amine; tris[4'-(diphenylamino)-1,1'-biphenyl-4-yl]amine; tris[4'-(carbazol-9-yl)-1,1'-biphenyl-4-yl]amine; tris[4'-(1-naphthylphenylamino)-1,1'-biphenyl-4-yl]amine; tris[4'-(phenyl-m-tolylamino)-1,1'-biphenyl-4-yl]amine; N,N-bis[4'-(phenyl-m-tolylamino)-1,1'-biphenyl-4-yl]-N'-phenyl-N'-m-tolyl-3,3'-dimethylbenzidine; N,N-bis(4'-diphenylamino-1,1'-biphenyl-4-yl)-N'-phenyl-N'-m-tolyl-3,3'-dimethylbenzidine; N,N-bis(diphenylamino-1,1'-biphenyl-4-yl)-N'-phenyl-N'-m-tolylbenzidine; N,N-bis[4'-(di-m-tolylamino)-1,1'-biphenyl-4-yl]-N'-phenyl-N'-p-tolylbenzidine; tris[4'-(8H-10H-acridin-10-yl)-1,1'-biphenyl-4-yl]amine; tris[4'-(9,9-dimethyl-9H-10H-acridin-10-yl)-1,1'-biphenyl-4-yl]amine; tris[4'-phenoxy-10-yl-1,1'-biphenyl-4-yl]amine; tris[4'-phenoxy-10-yl-1,1'-biphenyl-4-yl]amine; N,N-bis[4'-(phenyl-m-tolylamino)-1,1'-biphenyl-4-yl]-N'-phenyl-N'-m-tolylbenzidine; N,N-bis[4'-(1-naphthylphenylamino)-1,1'-biphenyl-4-yl]-N'-carbazol-9-yl)-1,1'-biphenyl-4-amine; and N,N-bis[4'-(9H-10H-acridin-10-yl)-1,1'-biphenyl-4-yl]-N'-carbazol-9-yl)-1,1'-biphenyl-4-amine.

\* \* \* \* \*